# EUROPEAN PATENT SPECIFICATION

(11) **EP 2 855 772 B1**
(45) Date of publication and mention of the grant of the patent: **08.06.2016**
(21) Application number: 13723935.6
(22) Date of filing: 17.05.2013
(51) Int. Cl.: D21H 27/00, D21H 17/25, D21H 19/34, D21H 21/16, D21H 21/18

(54) **A SUBSTRATE FOR SECURITY DOCUMENTS**
EIN SUBSTRAT FÜR SICHERHEITSDOKUMENTE
SUBSTRAT POUR DES DOKUMENTS DE SECURITES

(30) Priority: 29.05.2012 GB 201209516
(43) Date of publication of application: 08.04.2015
(73) Proprietor: De La Rue International Limited, Basingstoke, Hampshire RG22 4BS (GB)
(72) Inventor: RATNAKUMAR, Rohan, Basingstoke Hampshire RG21 8XQ (GB); HOWLAND, Paul, Andover Hampshire SP10 2QR (GB)
(74) Representative: Boult Wade Tennant
(86) International application number: PCT/GB2013/051282
(87) International publication number: WO 2013/178986

(56) References cited:
- EP-A1- 0 198 837
- WO-A1-2008/054581
- WO-A1-2011/056130
- WO-A1-2011/068457
- WO-A2-2012/098296
- GB-A- 2 066 145

## Description

The present invention provides a durable substrate for security documents such as banknotes, cheques, identification documents etc. and a method of manufacturing such a substrate. In particular, the present invention relates to durable substrates that are resistant to the build-up of soil on their surfaces, thereby reducing the rate at which documents are out-sorted by sorting machines or otherwise rejected for further use as information provided on the document becomes unreadable.

Security documents such as banknotes, identification documents and other such multi-use documents are subjected to regular handling and storage in places in which soil (e.g. oils and dirt)can accumulate and be transferred to the surface of the document. Soil can eventually build up to such an extent as to render security features or security information provided thereupon difficult to read by either human or machine scrutiny. At this point, the document must be taken out of circulation, destroyed and replaced, at a cost borne by the bearer or the bank note issuing authority.

Durable security documents are already known. Banknotes in some countries, such as Australia and Canada, are printed on polymeric substrates which have an enhanced lifespan over conventional paper-based substrates. Whilst these polymeric substrates offer improved physical durability, this comes with a number of disadvantages, such as increased initial manufacturing costs and the increased complexity in trying to incorporate certain types of security devices, which would be incorporated into paper-based substrates at the time of their manufacture, e.g. watermarks, embedded or windowed security elements etc.. Additionally polymer substrates have a polymer tactility, which means that such banknotes no longer have the traditional feel and sound of a banknote.

Composite paper-polymer substrates are also known in the art, and laminar substrates having paper-polymer-paper or polymer-paper-polymer structures are commercially available. These go some way to addressing the security limitations of purely polymer-based substrates, but again at very high manufacturing costs. Furthermore they can suffer particularly in humid environments where differences in hygro-expansivity between the paper and polymeric layers result in inherent weaknesses in the laminar substrate that present opportunities to the counterfeiter.

Soil-resistant traditional paper security substrates are also commercially available, such as the Platinum®-coated paper made by De La Rue (UK), or the AST-coated paper from Crane & Co (USA). In these systems, synthetic polymer-based soil-resistant coatings are applied to the surface of the substrate to size and seal it against the ingress of oils and dirt encountered in circulation.

While all of these approaches go some way to solving the problem of providing durable security substrates, there still remains a need for documents with enhanced circulation lifetimes. In particular, there still remains a need for security substrates having improved soil resistance and physical integrity combined with reduced environmental impact including end-of-life biodegradability or facile re-pulping of production spoil.

As cellulose is one of the most commonly found natural polymers, much research has been carried out over the years into ways of processing cellulose fibres to improve their usefulness. This lead to research into microfibrillating cellulose. Microfibrillation is the process of opening up the fibre structure to increase the surface-to-volume ratio thereof. It also results in the shortening of the fibres, resulting in a fine particle size of the order of micrometres to tens of micrometres such that the microfibrils exhibit a gel-like characteristic in water with pseudo plastic and thixotropic properties. The manufacture of microfibrillated cellulose (MFC) first came about in the late 1970s. However the aforementioned properties make MFC a difficult material to handle so commercial uses of MFC have been slow to develop.

In the packaging industry, it has been found that MFC enhances the properties of a water vapour barrier of a dispersion coating made from colloidal particles of a polymer. This is described in WO-A-2011/056130. The addition of the MFC to the dispersion coating has been shown to improve the water holding capacity and reduces the brittleness of the coating.

WO-A-2011/078770 describes the use of MFC in a layered arrangement to provide a paper or paperboard substrate having barrier properties against liquids, vapour and gases. To provide this the paper or paperboard substrate has a first fibre based layer, a second layer comprising MFC and a third layer comprising a polymer. The MFC layer is provided to increase the density of the fibre layer and to smooth the surface thereof, which in turn increases the smoothness and
the adherability of the polymer layer which provides the known barrier to liquids/vapour. It has been found that the combination of the MFC and the polymer layers provides good oxygen barrier properties which are not provided by the use of the polymer coating by itself.

The prior art is concerned with using MFC as part of a polymer based barrier coating. Polymer based barrier coatings are not ideal for use on security documents particularly as a coating for a security paper which is to be printed on as the time taken for typical security inks to dry (oil based lithographic and intaglio inks) will be slower than on paper where the ink can be absorbed into rough paper surface.

EP-A-0198837 discloses paper with improved surface properties, especially printability and coating properties. The invention is characterized in that the paper comprises a surface layer consisting of highly beaten paper pulp, fine material or fibres separated from highly beaten paper pulp and/or fine material, possibly containing fibres, from white water, in an amount of at maximum 10 g/m², preferably at maximum 5 g/m².

WO-A-2008/054581 discloses a soil and/or moisture resistant secure document and a method for producing such a secure document. The inventive method preferably employs a size press or other similar device to force a soil and/or moisture resistant formulation into the pores of the substrate and to remove excess formulation from opposing surfaces thereof. Soil and/or moisture resistant formulations when applied this way instead of by way of standard coating techniques do not obscure optically variable effects generated by nonporous OVDs that may be employed on or within these secure documents. In addition, thin layers of fibers (e.g. papermaking fibers) overlying and thus embedding portions of security devices in windowed secure documents that have been rendered soil and/or moisture resistant in accordance with this invention demonstrate increased durability.

WO-A-2011/068457 discloses a process for producing a paper or paperboard product which process comprises the steps of, providing a furnish comprising fibers, adding starch to the furnish, adding microfibrillated cellulose to the furnish, conducting the furnish to a wire in order to form a web, wherein the starch and microfibrillated cellulose is added separately to the furnish.

Thus the use of MFC is known in the paper and paperboard industry for some limited applications as described above. The present invention has arisen through the surprising discovery that, when used by itself with a paper substrate, and not in conjunction with a polymer layer, it advantageously provides an unexpected level of soil resistance. In addition the use of the MFC material in this manner enable the characteristics of the paper surface to be maintained which provides the improved soil resistance without significantly impacting on the ink drying characteristics of the security paper.

The invention lies in the use of a particular form of cellulose fibre known as microfibrillated cellulose (MFC), which is incorporated into and/or applied to the surface of a paper substrate, to improve the strength of security documents, such as banknotes, made from the substrate and to reduce their uptake of soil due to day to day handling.

The invention therefore provides a soil resistant paper substrate made from a stock comprising a suspension of paper fibres and treated with microfibrillated cellulose such that the microfibrillated cellulose bridges pore spaces formed by and in between the paper fibres at at least a surface of the substrate to provide soil resistance.

The microfibrillated cellulose may be added to the stock, and/or applied to the substrate prior to printing and/or after printing.

The invention further comprises a security paper formed from the aforementioned soil resistant paper comprising an overt security feature to which a transparent microfibrillated cellulose based soil resistant coating or varnish is applied.

The invention additionally comprises a security document comprising the aforementioned soil resistant paper substrate wherein the document is printed before the microfibrillated cellulose is applied as a coating to the surface of the substrate.

The invention also comprises a method of manufacturing a soil resistant paper substrate comprising the steps of forming an intermediate paper substrate from a stock comprising suspension of paper fibres and coating the substrate with a coating comprising microfibrillated cellulose such that the microfibrillated cellulose bridges pore spaces formed by and in between the paper fibres at at least a surface of the substrate to provide soil resistance.

The invention further comprises a method of manufacturing a soil resistant paper substrate comprising the step of adding microfibrillated cellulose to a stock comprising a suspension of paper fibres and forming the substrate such that the microfibrillated cellulose bridges pore spaces formed by and in between the paper fibres at at least a surface of the substrate to provide soil resistance.

The aforementioned problems are thus substantially addressed by the present invention. The microfibrillated cellulose (MFC) has the advantage that it is inherently low cost compared to polymer coatings as it is produced from a common raw material, such as wood or cotton pulp, rather than by a complex chemical synthesis process based on petrochemicals.

Because of its surprising ability to bridge the inherent surface pore structure of paper, significantly less MFC coating is required in order to obtain the same effect as an equivalent polymer coating which provides a processing benefit. This is due to the fibril nature of the MFC which enables it to bridge the pore structure of the paper. Unlike with the known polymer based soil resistant coatings, the MFC coatings of the current invention will not flow into the paper substrate when heated and therefore all of the MFC will be used to bridge the pore structure and therefore improve the soil resistance. With the polymer coating, on the other hand, a significant volume of the coating will flow into the paper structure and only fraction will function as a soil resistant coating on the surface.

Similarly, when MFC is incorporated into the substrate during the paper making process (rather than by means of a coating process which requires additional processing steps), this leads to a reduction in the porosity of the substrate, which improves the resistance of the substrate to soil compared to paper made in the usual way.

Advantageously, with the MFC consisting predominantly of physically-modified cellulose, it undergoes the same biological degradation as the bulk cellulose of the substrate, and spoil can be incorporated directly back into papermaking stock by standard re-pulping processes.

Methods for producing microfibrillated cellulose are described in, for example, GB-A-2066145, in which a liquid suspension of cellulose at high pressure is passed through an orifice to cause an explosive decompression of the suspension and the fibres contained therein. Unfortunately, the energy expenditure required to produce MFC's by mechanical means is very high, requiring approximately 30000kWh/tonne of product. Alternative approaches are described in, inter alia, WO-A-2007/091942, which discloses an enzymatic process by which microfibrillation of wood pulp can be performed, resulting in a product comparable to that described in GB-A-2066145 but at drastically reduced energy expenditure. The MFC's of the present invention can be prepared from any source of cellulosic material, including wood pulp or preferably cotton fibres. Wood pulp contains 40-50% cellulose, while cotton fibres contain up to around 90% cellulose.

The cellulose found in cotton fibre shows a higher degree of polymerisation in comparison to cellulose derived from other natural fibres and especially soft and hard wood pulps. The combination of higher degree of polymerisation and the higher cellulose content makes it generally harder for the micro fibrillation or homogenisation to easy generate MFC from cotton. Due to the process difficulties cotton would not be a natural choice of base material for generation of MFC.

The following table gives some typical values for the dimensions of cellulose fibres prior to, and following, the above cited microfibrillation process:

| | Length | Width | Thickness |
|---|---|---|---|
| Non-microfibrillated Cotton | 0.8-1.2 mm | 10-20 µm | 3-20 µm |
| Microfibrillated Cellulose | 1-100 µm | 5-10 nm | 5-10 nm |

The length of the fibres in the MFC may be up to 100µm, and preferably 50µm or less and is most preferably 10µm or less.

The width of the fibres in the MFC may be in the range 1 to 100nm, preferably 2 to 50nm, preferably 5 to 20nm and most preferably approximately 5nm.

The thickness of the fibres may lie in the range 2 to 50nm, preferably 5 to 20nm and is most preferably approximately 5nm.

Note in particular the three or more orders of magnitude by which all of the dimensions of the fibres are reduced during the process.

In one embodiment of the present invention, MFC is used as a coating applied to the external surface of a paper substrate, to provide a substrate from which security documents, such as banknotes can be made, in order to increase soil resistance. Traditionally used polymer-based coatings require a coat weight of approximately 2 grammes/m² (gsm) to provide a soil index of 15-30%. Using MFC, a similar level of soil resistance can be obtained by a significantly lower coat weight in the range of 0.1 to 5gsm, preferably 0.5 to 3gsm and is most preferably 1gsm. In the present context, the soil index is defined as the ratio of the differences in the luminosities of uncoated and coated substrates, subjected to standard soiling procedures, expressed as a percentage. The skilled practitioner will be familiar with the so-called FIRA (Furniture Industry Research Association) Soil test, referred to in WO-A-9628610. In this test, a sample of the paper is placed at one end of a cylinder along with a reference sample placed at the opposite end and 20 felt cubes impregnated with artificial sweat and colloidal graphite. The cylinder is rotated in alternate directions for a period of 30 minutes. The change in reflectance of the printed samples is measured and the relative soil pickup is calculated by comparing the results of the test. In such tests, soil-resistant substrates such as Platinum^{®}-coated paper supplied by De La Rue (United Kingdom) and AST^{®} Paper supplied by Crane & Co (USA) achieve soil indices of between 20-30%. The MFC coated paper substrate of the present invention achieves an equivalent soil index.

It is believed that the microfibrillated cellulose, with its chemically identical structure, has stronger interactions with, and is more efficient at bridging, the pores between the non-microfibrillated fibres of the substrate than the polymeric coatings typically employed. This means that the number of loose fibre ends and the overall surface area of the substrate is reduced, producing a concomitant reduction in soiling. The MFC becomes crystalline as it cures, which helps to seal the pores and to resist oil based soil. Furthermore, the elimination of the differences in hygroscopicity between the coating and the substrate resolves the weaknesses in existing laminar security substrates identified above.

Paper derives its mechanical strength from hydrogen bonding between cellulose microfibrils. The MFC, which is also cellulose, will also have the ability to form hydrogen bonds, not only between the nanofibrils of the MFC but with the cellulose microfibrils of the paper fibres. It will therefore adhere well to the base paper fibres.

MFC can be applied to a paper substrate by any known coating method such as doctor blades, dip roll coating, gravure, flexography etc. with dip coating and gravure being preferred techniques. The MFC is typically delivered to the substrate as a suspension of fibres, preferably in an aqueous medium, the suspension having a solids content of approximately 3% weight for weight (w/w). A particular advantage of using MFC as a coating on a secure paper substrate is that coatings produced from suspensions having a solids content in the range 0.1 to 30% weight for weight (w/w), and preferably in the range 2 to 15% weight for weight (w/w), are transparent and therefore do not affect the appearance of security features incorporated into the paper substrate such as watermarks or embedded or partially embedded security threads. In addition to additional coating methods the MFC can be delivered to the substrate using a size press in line on a paper machine. In this case the MFC is mixed with water to obtain an aqueous formulation having a solids content ranging from about 1-30% dry weight, and more preferably 1-10% dry weight.

In a second embodiment of the present invention, MFC is incorporated throughout the body of the paper substrate by mixing it with standard cotton fibre stock in the papermaking stage of production. In a typical example, the addition of 10% MFC to the bulk of a cotton fibre-based substrate affords a soil index according to the same test as described above of the order of 15%. The stock is preferably formed by adding microfibrillated cellulose to the suspension of paper fibres in a quantity of up to 30% by weight. The MFC is a suspension of fibres in an aqueous medium which preferably has a solids content of 0.01 to 1% w/w, and more preferably 0.05 to 0.5% w/w.

In a third embodiment of the present invention, MFC is used as a post-print varnish to further improve the circulation durability of security documents coated therewith. Printing inks are formulated to optimise their adhesion to the substrate onto which they are to be printed. As the cotton-based substrate and the MFC-based post-print varnish share identical chemistries, the adhesion between varnish, ink and substrate is also optimised. Post-print varnishes may be applied by any suitable coating technique known to the skilled practitioner. Preferred techniques include flexography, which can be used to deposit coat weights of approximately 1gsm from a 3% w/w suspension of MFC. The formulation of the MFC coating must be selected to be sufficiently transparent not to detract from the underlying print and other security features on the finished security document. A coat weight of approximately 1gsm from a 3% w/w suspension of MFC would be transparent. The preferred range for the solids content of the suspension of MFC would be from 0.1 to 30% w/w, and more preferably 2 to 15% w/w.

The fibres which are present in the initial paper stock may be all natural fibres or a mixture of natural and synthetic fibres, or all synthetic fibres. The fibres used may be, for example, PVOH, Polyamide, polyester, or other poly olefins.

Although the principal required benefit of using MFC in the present invention is to provide improved soil resistance, it was also found that as the ratio of MFC used in, or added to, the paper was increased, there was a consequential increase in the strength of the paper substrate, a decrease in porosity and an improvement in double folds tests. Double fold tests measure the durability of paper when repeatedly folded under constant load. A Schopper double fold tester may be used to determine the number of times a paper can be folded until it breaks. The folding strength is quoted as the number of double folds until the paper breaks (at 23C and 50% RH).

These improvements are illustrated by the test results given below.

The following results were obtained in hand tests on 90gsm hand sheets formed using waterleaf paper stock and MFC. Separate batches of MFC were formed from cotton pulp and wood pulp respectively, and these were added to separate batches of the paper stock in different proportions (0, 5, 10, 15 and 20% w/w as illustrated in the tables below. The MFC was diluted to provide a gel comprising 0.15 - 0.17% microfibrils in water.

**Wood Pulp MFC**

| % | g | g | M1 | ml |
|---|---|---|---|---|
| **MFC addition rate** | **Dry wt of hand sheet** | **MFC dry wt/sheet** | **Vol of MFC to add @ 0.15%** | **Vol of stock used** |
| 0 | 1.8 | 0 | 0 | 460 |
| 5 | 1.8 | 0.09 | 60 | 435 |
| 10 | 1.8 | 0.18 | 120 | 410 |
| 15 | 1.8 | 0.27 | 180 | 385 |
| 20 | 1.8 | 0.36 | 240 | 360 |

**Cotton Pulp MFC**

| % | g | g | M1 | ml |
|---|---|---|---|---|
| **MFC addition rate** | **Dry wt of hand sheet** | **MFC dry wt/sheet** | **Vol of MFC to add @ 0.15%** | **Vol of stock used** |
| 0 | 1.8 | 0 | 0 | 425 |
| 5 | 1.8 | 0.09 | 60 | 405 |
| 10 | 1.8 | 0.18 | 120 | 385 |
| 15 | 1.8 | 0.27 | 180 | 365 |
| 20 | 1.8 | 0.36 | 240 | 345 |

Eight sheets of each were dried and subjected to tensile strength, double folds and porosity tests with the average results shown below.

The Bendtsen test is a standard test and we can quote ISO 5636-3

| **MFC %** | **0** | **5** | **10** | **15** | **20** |
|---|---|---|---|---|---|
| Bendtsen Porosity (ml/min) | 107.7 | 45.7 | 26.7 | 6.7 | 3.3 |
| Double Folds | 2091 | 1327 | 2476 | 2335 | 2895 |
| Tensiles (KgF) | 7.2 | 6.5 | 10.1 | 10.0 | 11.1 |

**Cotton Pulp MFC**

| **MFC %** | **0** | **5** | **10** | **15** | **20** |
|---|---|---|---|---|---|
| Bendtsen Porosity (ml/min) | 120 | 77 | 35 | 15 | 6 |
| Double Folds | 996 | 2652 | 2158 | 3290 | 3267 |
| Tensiles (KgF) | 7.2 | 7.9 | 9.1 | 10.1 | 11.5 |

The increase in the strength of the paper substrate and the improvement in the results from the double-folds test were more significant when cotton based MFC were added to the stock compared to wood based MFC. The additional strength benefits from the cotton based MFC reduces the creation of pores in the paper substrate when in circulation as a banknote or other secure substrate. A reduction in pores leads to a reduction in soiling as the soil tends to accumulate in pores on the surface of a banknote or secure substrate.

In further embodiments MFC can be incorporated both in the stock and applied as a pre-print or post-print coating. In this case the pre-print coating can be applied using a size press.

Additional soil resistant layers can also be coated onto the paper. This could take the form of a conventional pre-print coating which are typically aqueous resin binder systems such as those based on polyurethane dispersions and as described in EP-A-0815321. A typical example is Platinum^{®} as sold by De La Rue International Limited. Alternatively a size press can be used to apply the coating as is known from EP-A-2074260. For example polyether-polyurethane resin based systems are typically used for the size press. The application of a conventional pre-print anti-soil coating over a paper substrate with MFC incorporated into the stock results in a surprisingly significant improvement in soil resistance over that observed without the MFC incorporated into the stock.

In one example paper stock was formed by adding cotton derived MFC to the suspension of paper fibres in a quantity of 15% by weight. The resulting paper was further coated with a size press, as described in EP-A-2074260, using an aqueous formulation from a selection of thermoplastic resins such as resins having an ester bond (e.g. polyester resins and polyether resins), polyurethane resins, functionalized polyurethane resins (e.g. carboxylated polyurethane resins), and copolymers (e.g.urethane-acrylic resins, polyether-urethane resins and styrene acrylate resins) and mixtures thereof. Alternatively the paper was coated with a Platinum^{®} polyurethane using materials and techniques described in EP-A-0815321. The coat weight of such a polyurethane coating will be between 0.05 and 20 gsm and more preferably between 0.5 and 5gsm.

An improvement in soil resistance was observed when the MFC is incorporated both into the paper substrate and then applied as a coating using a size press. For example, paper stock was formed by adding cotton derived MFC to the suspension of paper fibres in a quantity of 15% by weight and then sized with cotton derived MFC with a consistency of approximately 2% on a dry weight basis using a size press. The size is made by mixing the cotton derived MFC with water so as to form an aqueous formulation having a solids content of 2% by dry weight. Surprisingly a significant further improvement in soil resistance was obtained if the resultant paper was then coated with an additional soil resistant layer, for example with a 2gsm dry coating of a formulation of polyurethane dispersion, such as Platinum^{®}. The combination of MFC in the paper stock and then application of MFC using a size press followed by a conventional polyurethane soil resistant coating produced a 50% enhancement of the soil resistance compared to that typically achieved by conventional polyurethane products.

This improvement could be explained by the effective closure of micro pores within the paper by MFC. This would reduce the amount of the additional soil resistant layer, such as a conventional polyurethane coating, that would penetrate into the pore in the paper and therefore more of the coating is available on the surface. This results in a more coherent film of polyurethane formation on the surface reducing soil penetration and accumulation.

## Claims

1. A soil resistant security paper substrate for banknotes made from a stock comprising a suspension of paper fibres, and microfibrillated cellulose, the microfibrillated cellulose bridging pore spaces formed by and in between the paper fibres at at least a surface of the substrate to provide soil resistance, **characterised in that** the microfibrillated cellulose is produced from cotton pulp and **in that** the length of fibres in the microfibrillated cellulose lies in the range 1 to 100µm and the width of said fibres lies in the range of 2 to 50nm.

2. A method of manufacturing a soil resistant security paper substrate for banknotes comprising the step of adding microfibrillated cellulose to a stock comprising a suspension of paper fibres and forming the substrate, wherein the microfibrillated cellulose bridges pore spaces formed by and in between the paper fibres at at least a surface of the substrate to provide soil resistance, **characterized in that** the microfibrillated cellulose is produced from cotton pulp and **in that** the length of fibres in the microfibrillated cellulose lies in the range 1 to 100µm and the width of said fibres lies in the range of 2 to 50nm.

3. A soil resistant security paper substrate for banknotes or a method of manufacturing a soil resistant security paper substrate for banknotes as claimed in any one of the preceding claims in which the microfibrillated cellulose is added to the stock as a suspension of fibres in an aqueous medium which suspension has a solids content of 0.01 to 1% weight for weight, and preferably 0.05 to 0.5% weight for weight.

4. A soil resistant security paper substrate for banknotes or a method of manufacturing a soil resistant security paper substrate for banknotes as claimed in any one of the preceding claims in which the microfibrillated cellulose is added to the stock in a quantity of up to 30% by weight.

5. A soil resistant security paper substrate for banknotes or a method of manufacturing a soil resistant security paper substrate for banknotes as claimed in any one of the preceding claims in which the microfibrillated cellulose is applied as a coating to the surface of the substrate after formation of an intermediate paper substrate from the paper fibre suspension.

6. A soil resistant security paper substrate for banknotes or a method of manufacturing a soil resistant security paper substrate for banknotes as claimed in claim 5 in which the microfibrillated cellulose coating is applied by means of a size press.

7. A soil resistant security paper substrate for banknotes or a method of manufacturing a soil resistant security paper substrate for banknotes as claimed in claim 5 or claim 6 in which the microfibrillated cellulose coating is applied to the surface of the substrate after the substrate has been printed.

8. A soil resistant security paper substrate for banknotes or a method of manufacturing a soil resistant security paper substrate for banknotes as claimed in any one of claims 5 to 7 in which the coat weight of the microfibrillated cellulose coating lies in the range 0.1 to 5gsm, and preferably 0.5 to 3 gsm and is most preferably 1 gsm.

9. A soil resistant security paper substrate for banknotes or a method of manufacturing a soil resistant security paper substrate for banknotes as claimed in any one of claims 5 to 8 in which the microfibrillated cellulose coating is a suspension of fibres in an aqueous medium, the suspension having a solids content of 0.1 to 30% weight for weight, and preferably 2 to 15% weight for weight.

10. A soil resistant security paper substrate for banknotes or a method of manufacturing a soil resistant security paper substrate for banknotes as claimed in any one of the preceding claims in which the length of the fibres in the microfibrillated cellulose is up to 50µm and more preferably up to 10µm.

11. A soil resistant security paper substrate for banknotes or a method of manufacturing a soil resistant security paper substrate for banknotes as claimed in any one of the preceding claims in which the width of the fibres in the microfibrillated cellulose lies in the range 5 to 20nm, and is preferably 5nm.

12. A soil resistant security paper substrate for banknotes or a method of manufacturing a soil resistant security paper substrate for banknotes as claimed in any one of the preceding claims in which the thickness of the fibres in the microfibrillated cellulose lies in the range 1 to 100nm, preferably 2 to 50nm, preferably 5 to 20nm, and is most preferably 5nm.

13. A security paper formed from the soil resistant security paper substrate for banknotes as claimed in claim 1 or any one of claims 3 to 12 as dependent upon claim 1 comprising an overt security feature to which a transparent microfibrillated cellulose based soil resistant coating or varnish is applied.

14. A security document comprising the soil resistant security paper substrate for banknotes as claimed in claim 1 or any one of claims 3 to 13 as dependent upon claim 1 wherein the document is printed before a microfibrillated cellulose coating is applied to the surface of the substrate.

15. A method of manufacturing a soil resistant security paper substrate for banknotes as claimed in claim 2 or any one of claims 3 to 12 as dependant on claim 2 further comprising the step of applying an additional soil resistant layer.

16. A method of manufacturing a soil resistant security paper substrate for banknotes as claimed in claim 15 in which the additional soil resistant layer is applied before the substrate is printed.

17. A method of manufacturing a soil resistant security paper substrate for banknotes as claimed in claim 15 in which the additional soil resistant layer is applied after the substrate has been printed.

## Patentansprüche

1. Schmutzabweisendes Sicherheitspapiersubstrat für Banknoten hergestellt aus einem Material umfassend eine Suspension aus Papierfasern und mikrogefaserter Zellulose, wobei die mikrogefaserte Zellulose Porenräume an mindestens einer Oberfläche des Substrats überbrückt, die durch und zwischen den Papierfasern gebildet sind, um Schmutzabweisung bereit zu stellen, **dadurch gekennzeichnet, dass** die mikrogefaserte Zellulose aus Zellulosebrei hergestellt ist und dass die Länge der Fasern in der mikrogefaserten Zellulose in dem Bereich von 1 bis 100 µm liegt und die Breite der Fasern in dem Bereich von 2 bis 50 nm liegt.

2. Verfahren zur Herstellung eines schmutzabweisenden Sicherheitspapiersubstrats für Banknoten umfassend den Schritt eines Hinzufügens von mikrogefaserter Zellulose zu einem Material umfassend eine Suspension aus Papierfasern und Ausbilden des Substrats, wobei die mikrogefaserte Zellulose Porenräume an mindestens einer Oberfläche des Substrats überbrückt, die durch und zwischen den Papierfasern gebildet sind, um Schmutzabweisung bereit zu stellen, **dadurch gekennzeichnet, dass** die mikrogefaserte Zellulose aus Zellulosebrei hergestellt ist und dass die Länge der Fasern in der mikrogefaserten Zellulose in dem Bereich von 1 bis 100 mm liegt und die Breite der Fasern in dem Bereich von 2 bis 50 nm liegt.

3. Schmutzabweisendes Sicherheitspapiersubstrat für Banknoten oder Verfahren zur Herstellung eines schmutzabweisenden Sicherheitspapiersubstrats für Banknoten wie in irgend einem der vorhergehenden Ansprüche beansprucht, wobei die mikrogefaserte Zellulose zu dem Material als eine Suspension von Fasern in einem wässrigen Medium hinzugefügt wird, wobei diese Suspension einen Feststoffgehalt von 0.01 bis 1% Gewichtsanteil und bevorzugt 0.05 bis 0.5 % Gewichtsanteil aufweist.

4. Schmutzabweisendes Sicherheitspapiersubstrat für Banknoten oder Verfahren zur Herstellung eines schmutzabweisenden Sicherheitspapiersubstrats für Banknoten wie in irgend einem der vorhergehenden Ansprüche beansprucht, wobei die mikrogefaserte Zellulose zu dem Material in einer Menge von bis zu 30% Gewichtsanteil hinzugefügt wird.

5. Schmutzabweisendes Sicherheitspapiersubstrat für Banknoten oder Verfahren zur Herstellung eines schmutzabweisenden Sicherheitspapiersubstrats für Banknoten wie in irgend einem der vorhergehenden Ansprüche beansprucht, wobei die mikrogefaserte Zellulose als eine Beschichtung auf die Oberfläche des Substrats angewandt wird nach einer Bildung eines Zwischenpapiersubstrats aus der Papierfasersuspension.

6. Schmutzabweisendes Sicherheitspapiersubstrat für Banknoten oder Verfahren zur Herstellung eines schmutzabweisenden Sicherheitspapiersubstrats für Banknoten wie in Anspruch 5 beansprucht, wobei die mikrogefaserte Zellulosebeschichtung mittels einer Leimpresse angewandt wird.

7. Schmutzabweisendes Sicherheitspapiersubstrat für Banknoten oder Verfahren zur Herstellung eines schmutzabweisenden Sicherheitspapiersubstrats für Banknoten wie in Anspruch 5 oder Anspruch 6 beansprucht, wobei die mikrogefaserte Zellulosebeschichtung auf die Oberfläche des Substrats angewandt wird, nachdem das Substrat gedruckt wurde.

8. Schmutzabweisendes Sicherheitspapiersubstrat für Banknoten oder Verfahren zur Herstellung eines schmutzabweisenden Sicherheitspapiersubstrats für Banknoten wie in irgend einem der Ansprüche 5 bis 7 beansprucht, wobei das Flächengewicht der mikrogefaserten Zellulosebeschichtung in dem Bereich von 0.1 bis 5 gsm und bevorzugt 0.5 bis 3 gsm liegt und am meisten bevorzugt 1 gsm ist.

9. Schmutzabweisendes Sicherheitspapiersubstrat für Banknoten oder Verfahren zur Herstellung eines schmutzabweisenden Sicherheitspapiersubstrats für Banknoten wie in irgend einem der Ansprüche 5 bis 8 beansprucht, wobei die mikrogefaserte Zellulosebeschichtung eine Suspension aus Fasern in einem wässrigen Medium ist, wobei die Suspension einen Feststoffgehalt von 0.1 bis 30% Gewichtsanteil und bevorzugt 2 bis 15 % Gewichtsanteil aufweist.

10. Schmutzabweisendes Sicherheitspapiersubstrat für Banknoten oder Verfahren zur Herstellung eines schmutzabweisenden Sicherheitspapiersubstrats für Banknoten wie in irgend einem der vorhergehenden Ansprüche beansprucht, wobei die Länge der Fasern in der mikrogefaserten Zellulose bis zu 50 µm ist und bevorzugt bis zu 10 µm ist.

11. Schmutzabweisendes Sicherheitspapiersubstrat für Banknoten oder Verfahren zur Herstellung eines schmutzabweisenden Sicherheitspapiersubstrats für Banknoten wie in irgend einem der vorhergehenden Ansprüche beansprucht, wobei die Breite der Fasern in der mikrogefaserten Zellulose in dem Bereich von 5 bis 20 nm liegt und bevorzugt 5 nm ist.

12. Schmutzabweisendes Sicherheitspapiersubstrat für Banknoten oder Verfahren zur Herstellung eines schmutzabweisenden Sicherheitspapiersubstrats für Banknoten wie in irgend einem der vorhergehenden Ansprüche beansprucht, wobei die Dicke der Fasern in der mikrogefaserten Zellulose in dem Bereich von 1 bis 100 nm, bevorzugt 2 bis 50 nm, bevorzugt 5 bis 20 nm liegt und am meisten bevorzugt 5 nm ist.

13. Sicherheitspapier ausgebildet aus dem schmutzabweisenden Sicherheitspapiersubstrat für Banknoten wie in Anspruch 1 oder in irgend einem der Ansprüche 3 bis 12 in ihrem Rückbezug auf Anspruch 1 beansprucht umfassend ein offenkundiges Sicherheitsmerkmal, auf das eine transparente und auf mikrogefaserter Zellulose basierende schmutzabweisende Beschichtung oder Lackierung angewandt ist.

14. Sicherheitsdokument, das das schmutzabweisende Sicherheitspapiersubstrat für Banknoten wie in Anspruch 1 oder in irgend einem der Ansprüche 3 bis 13 in ihrem Rückbezug auf Anspruch 1 beansprucht umfasst, wobei das Dokument gedruckt ist, bevor eine mikrogefaserte Zellulosebeschichtung auf die Oberfläche des Substrats angewendet wird.

15. Verfahren zur Herstellung von schmutzabweisenden Sicherheitspapiersubstrat für Banknoten wie in Anspruch 2 oder in irgend einem der Ansprüche 3 bis 12 in ihrem Rückbezug auf Anspruch 2 beansprucht ferner den Schritt eines Anwendens einer zusätzlichen schmutzabweisenden Schicht umfassend.

16. Verfahren zur Herstellung von schmutzabweisenden Sicherheitspapiersubstrat für Banknoten wie in Anspruch 15 beansprucht, wobei die zusätzliche schmutzabweisende Schicht angewandt wird, bevor das Substrat gedruckt wird.

17. Verfahren zur Herstellung von schmutzabweisenden Sicherheitspapiersubstrat für Banknoten wie in Anspruch 15 beansprucht, wobei die zusätzliche schmutzabweisende Schicht angewandt wird, nachdem das Substrat gedruckt wurde.

## Revendications

1. Substrat de papier de sécurité résistant à la salissure pour des billets de banque réalisé à partir d'une pâte comprenant une suspension de fibres de papier et de la cellulose microfibrillée, la cellulose microfibrillée couvrant des espaces interstitiels formés par les fibres de papier et entre celles-ci au niveau d'au moins une surface du substrat pour assurer la résistance à la salissure, **caractérisé en ce que** la cellulose microfibrillée est produite à partir d'une pâte de coton et **en ce que** la longueur de fibres dans la cellulose microfibrillée se trouve dans la plage allant de 1 à 100 µm et la largeur desdites fibres se trouve dans la plage allant de 2 à 50 nm.

2. Procédé de fabrication d'un substrat de papier de sécurité résistant à la salissure pour des billets de banque comprenant l'étape consistant à ajouter de la cellulose microfibrillée à une pâte comprenant une suspension de fibres de papier et à former le substrat, dans lequel la cellulose microfibrillée couvre des espaces interstitiels formés par les fibres de papier et entre celles-ci au niveau d'au moins une surface du substrat pour assurer la résistance à la salissure, **caractérisé en ce que** la cellulose microfibrillée est produite à partir d'une pâte de coton et **en ce que** la longueur de fibres dans la cellulose microfibrillée se trouve dans la plage allant de 1 à 100 µm et la largeur desdites fibres se trouve dans la plage allant de 2 à 50 nm.

3. Substrat de papier de sécurité résistant à la salissure pour des billets de banque ou procédé de fabrication d'un substrat de papier de sécurité résistant à la salissure pour des billets de banque tel que revendiqué dans l'une quelconque des revendications précédentes, dans lequel la cellulose microfibrillée est ajoutée à la pâte sous forme de suspension de fibres dans un milieu aqueux, laquelle suspension a une teneur en matières solides comprise entre 0,01 et 1 % poids pour poids, et de préférence comprise entre 0,05 et 0,5 % poids pour poids.

4. Substrat de papier de sécurité résistant à la salissure pour des billets de banque ou procédé de fabrication d'un substrat de papier de sécurité résistant à la salissure pour des billets de banque tel que revendiqué dans l'une quelconque des revendications précédentes, dans lequel la cellulose microfibrillée est ajoutée à la pâte en une quantité allant jusqu'à 30 % en poids.

5. Substrat de papier de sécurité résistant à la salissure pour des billets de banque ou procédé de fabrication d'un substrat de papier de sécurité résistant à la salissure pour des billets de banque tel que revendiqué dans l'une quelconque des revendications précédentes, dans lequel la cellulose microfibrillée est appliquée en tant que revêtement à la surface du substrat après la formation d'un substrat de papier intermédiaire à partir de la suspension de fibres de papier.

6. Substrat de papier de sécurité résistant à la salissure pour des billets de banque ou procédé de fabrication d'un substrat de papier de sécurité résistant à la salissure pour des billets de banque tel que revendiqué dans la revendication 5, dans lequel le revêtement en cellulose microfibrillée est appliqué au moyen d'une presse encolleuse.

7. Substrat de papier de sécurité résistant à la salissure pour des billets de banque ou procédé de fabrication d'un substrat de papier de sécurité résistant à la salissure pour des billets de banque tel que revendiqué dans la revendication 5 ou 6, dans lequel le revêtement en cellulose microfibrillée est appliqué à la surface du substrat après que le substrat a été imprimé.

8. Substrat de papier de sécurité résistant à la salissure pour des billets de banque ou procédé de fabrication d'un substrat de papier de sécurité résistant à la salissure pour des billets de banque tel que revendiqué dans l'une quelconque des revendications 5 à 7, dans lequel le poids de revêtement du revêtement en cellulose microfibrillée se trouve dans la plage allant de 0,1 à 5 g/m², et de préférence de 0,5 à 3 g/m² et est plus préférablement de 1 g/m².

9. Substrat de papier de sécurité résistant à la salissure pour des billets de banque ou procédé de fabrication d'un substrat de papier de sécurité résistant à la salissure pour des billets de banque tel que revendiqué dans l'une quelconque des revendications 5 à 8, dans lequel le revêtement en cellulose microfibrillée est une suspension de fibres dans un milieu aqueux, la suspension ayant une teneur en matières solides comprise entre 0,1 et 30 % poids pour poids, et de préférence entre 2 et 15 % poids pour poids.

10. Substrat de papier de sécurité résistant à la salissure pour des billets de banque ou procédé de fabrication d'un substrat de papier de sécurité résistant à la salissure pour des billets de banque tel que revendiqué dans l'une quelconque des revendications précédentes, dans lequel la longueur des fibres dans la cellulose microfibrillée peut aller jusqu'à 50 µm et plus préférablement jusqu'à 10 µm.

11. Substrat de papier de sécurité résistant à la salissure pour des billets de banque ou procédé de fabrication d'un substrat de papier de sécurité résistant à la salissure pour des billets de banque tel que revendiqué dans l'une quelconque des revendications précédentes, dans lequel la largeur des fibres dans la cellulose microfibrillée se trouve dans la plage allant de 5 à 20 nm et est de préférence de 5 nm.

12. Substrat de papier de sécurité résistant à la salissure pour des billets de banque ou procédé de fabrication d'un substrat de papier de sécurité résistant à la salissure pour des billets de banque tel que revendiqué dans l'une quelconque des revendications précédentes, dans lequel l'épaisseur des fibres dans la cellulose microfibrillée se trouve dans la plage allant de 1 à 100 nm, de préférence de 2 à 50 nm, de préférence de 5 à 20 nm, et est plus préférablement de 5 nm.

13. Papier de sécurité formé à partir du substrat de papier de sécurité résistant à la salissure pour des billets de banque tel que revendiqué dans la revendication 1 ou l'une quelconque des revendications 3 à 12 lorsqu'elles dépendent de la revendication 1, comprenant un élément de sécurité explicite auquel est appliqué un revêtement ou un vernis transparent résistant à la salissure à base de cellulose microfibrillée.

14. Document de sécurité comprenant le substrat de papier de sécurité résistant à la salissure pour des billets de banque tel que revendiqué dans la revendication 1 ou l'une quelconque des revendications 3 à 13 lorsqu'elles dépendent de la revendication 1, dans lequel le document est imprimé avant l'application d'un revêtement en cellulose microfibrillée à la surface du substrat.

15. Procédé de fabrication d'un substrat de papier de sécurité résistant à la salissure pour des billets de banque tel que revendiqué dans la revendication 2 ou l'une quelconque des revendications 3 à 12 lorsqu'elles dépendent de la revendication 2, comprenant en outre l'étape consistant à appliquer une couche supplémentaire résistant à la salissure.

16. Procédé de fabrication d'un substrat de papier de sécurité résistant à la salissure pour des billets de banque tel que revendiqué dans la revendication 15, dans lequel la couche supplémentaire résistant à la salissure est appliquée avant que le substrat ne soit imprimé.

17. Procédé de fabrication d'un substrat de papier de sécurité résistant à la salissure pour des billets de banque tel que revendiqué dans la revendication 15, dans lequel la couche supplémentaire résistant à la salissure est appliquée après que le substrat a été imprimé.
